# EUROPEAN PATENT SPECIFICATION

(11) **EP 2 009 143 B1**
(45) Date of publication and mention of the grant of the patent: **09.08.2017**
(21) Application number: 07119756.0
(22) Date of filing: 31.10.2007
(51) Int. Cl.: C23C 18/16

(54) **Bipolar electroless deposition method**
Bipolares, stromloses Beschichtungsverfahren
Procédé des revetement bipolaire sans courant

(30) Priority: 08.05.2007 US 916771 P
(43) Date of publication of application: 31.12.2008
(73) Proprietor: IMEC, 3001 Leuven (BE)
(72) Inventor: Vereecken, Philippe M., B-4000 Liege (BE)
(74) Representative: Pronovem

(56) References cited:
- GB-A- 2 097 820
- US-A- 3 075 892
- US-A- 4 009 297
- US-A1- 2005 023 248
- US-A1- 2006 166 474

## Description

### FIELD OF THE INVENTION

The present disclosure is related to the field of bipolar electrochemical processing (Bi-ECP).

More specifically, the present invention is related to bipolar electroless processing.

The invention is particularly related to a method for selective electrochemical deposition of metallic particles onto a substrate.

The present invention further relates to specific uses of a method for selective deposition of metallic nanoparticles.

### BACKGROUND OF THE INVENTION

Electrochemical deposition (or plating) methods are widely used to deposit metallic compounds onto a surface of a substrate. Both electroplating and electroless plating processes are attractive methods to deposit pure metals or alloys from metal ions in solution. Besides (metal) deposition, also electrochemical metal-removal processes are widely used and applied for electro polishing, chemical etching and electro etching.

As such, in prior art, electrochemical metal deposition is explored as one of the methods for "selective" particles placement. The placement of metal nanoparticles on e.g. silicon (Si) substrates can be done by conventional electrochemical deposition (i.e. using an external power supply) directly on the substrate.

In conventional electrochemical processing (such as electrodeposition or electro etching) an external voltage and current is applied between at least two electrodes in an electrolyte bath. One half reaction (e.g. metal deposition through metal ion reduction) proceeds at the substrate or first electrode (work piece), and a second half reaction or counter reaction proceeds at a second electrode (current collector).

The control of said half reactions is a difficulty while working with conventional electrochemical processes using external voltage and current.

Furthermore, for the direct placement of metal nanoparticles on the substrate done by conventional electrochemical deposition, a contact needs to be made to the back side of the substrate (wafer). This can be done for example by pressing the back side of the substrate to a metal plate to obtain intimate contact and thus keep the contact resistance at a minimum. Also preferentially the back side of the substrate should be highly doped (e.g. by implantation) and additionally a suitable metal (that forms an ohmic contact with the Si substrate), metal silicide or metal germanide is coated on the substrate back side to minimize the contact resistance. However, in semiconductor processing, contamination of the substrate back side is a possible issue.

Electroless deposition can avoid the use of such a contact to the substrate. However, in conventional "chemical" electroless deposition, where the metal ion solution or electrolyte further contains a reducing agent, the surface needs to be first activated with a catalyst cluster such as Pd catalyst cluster particles for the out-plating of the metal on the catalyst. Obviously this method is not suitable for the deposition of nanoparticles which need to be as small or even smaller in size as the catalyst cluster particles themselves.

Further on, in electroless deposition by galvanic displacement the surface does not need to be activated first, but plays the role of reducing species instead. Electroless deposition by galvanic displacement is characterized by a process with two half reactions: a cathodic half reaction or reduction of metal ions to form the metal clusters on the substrate surface (e.g. Si) and the anodic half reaction or the oxidation of the substrate (e.g. Si). The partial currents of both half reactions have to be equal so that no effective external current flows, i.e. the reaction occurs electroless.

The total reaction for electroless deposition by galvanic displacement is spontaneous (free enthalpy ΔG < O), which means that the substrate has to be less noble than the metal which is deposited (also metal ion concentration and complexation determine ΔG).

In the case of semiconductor substrates, there is the additional requirement that the empty electron levels (LUMO) of the metal ions overlap with the valence band of the semiconductor (for deposition in the dark).

Electroless deposition by galvanic displacement means that both reduction (e.g. deposition) and oxidation occur at the same surface. This has many implications for the quality of the deposited metal and metal substrate interface. For example when metal particles or films are deposited on a blanket Si surface, the silicon surface itself will be oxidized (i.e. forming insulating SiO₂) unless HF is added to remove the oxide which is, however, not always practically possible.

A potential drawback (or advantage, depending on the application), of electroless deposition by galvanic displacement (on the same surface) is that the deposition can be self-limiting when one of the half reactions is shutdown. Self-limitation happens when the substrate surface is completely covered and thus the underlying substrate (which is also the reducing species) is not longer available to sustain the reaction. This typically happens when either an insoluble surface oxide is formed (e.g. SiO₂ on Si substrate) during the oxidation reaction or when the surface becomes fully covered by a dense metal layer as a result of the reduction (deposition) reaction. Hence, the self-limitation can be beneficial when only small particles or dense thin films are desired, but are a drawback when oxide-free surfaces and thick (dense) films are required.

Galvanic displacement reactions are used for thick metal deposits (e.g. Ni on Si as described by Niwa et al. Electrochimica Acta 48 (2003) 1295-1300), but these films are porous so that contact between substrate and solution is maintained.

Electroless deposition by galvanic displacement can also be used for selective deposition in patterns. However, here the issue is that the anodic and cathodic half reactions may randomly occur separately into different pattern features, such as holes: deposition may occur in one series of holes whereas the anodic counter reaction occurs in another set of holes. In this case, a galvanic cell is created where the half reactions are uncontrollably separated (in analogy with galvanic corrosion). This affects the yield of deposition and limits the use of electroless deposition for electrodeposition on patterned substrates.

In electroless processing, both half reactions (reduction and oxidation) occur simultaneous at one and the same substrate and no external voltage or current flow is necessary.

In bipolar electrochemistry, both half reactions also (as for electroless deposition) occur at one and the same substrate but the cathodic and anodic reactions are space separated by placing the substrate in an electric field applied between two feed electrodes. In this case no physical connection is made between the substrate and the power source. However, to drive the electrochemical reactions an external voltage and current need to be applied.

Bipolar electrochemistry, like conventional electrochemistry, requires a solution that can support the separate oxidation and reduction reactions i.e. an electrolyte. The electrolyte composition affects the electrolyte's conductivity and the electrochemistry on the isolated substrate.

Bipolar electrochemistry can be categorized into one of two arbitrary designations. First there is "open" bipolar electrochemistry and second there is "closed" bipolar electrochemistry.

Open bipolar electrochemistry occurs on an electrically and physically isolated substrate that is completely immersed in one suitable electrolyte.

In closed bipolar electrochemistry the substrate forms a barrier between the electrodes and separates the electrolyte into separate areas. The end result is that the electrolyte acts as an electrolytic wire between the feeder electrodes and the substrate.

A well-known example of closed bipolar electrochemistry can be found in fuel. In this case the chemical energy difference between the two electrolytes physically separated by an electrode provides the voltage difference and current supplied by the batteries.

In general, all known cases of bipolar electrochemistry have two terminal external electrodes in place, and hence can be designated as "electrolytic" bipolar electrochemical processes.

In closed bipolar electrochemistry the potential across the substrate is equal to the potential applied across the feeder electrodes, and electrochemistry will occur on the isolated substrate at relatively low field intensities.

In contrast, in open bipolar electrochemistry the applied electrical field must reach a minimum value, which is relatively large, before the onset of bipolar electrochemistry on the isolated substrate.

In conclusion, all available electrochemical deposition techniques in prior art as described above, in particular the use of bipolar electrodeposition or electroless deposition by galvanic displacement, still have drawbacks and limitations among others being self-limitation and low yield.

### AIMS OF THE INVENTION

The present invention aims to provide bipolar electroless processing methods, which do not present the drawbacks of the prior art techniques.

In particular, the present invention aims to deal with further optimalization towards a non-limiting and high-yield electrochemical deposition technique.

A preferred aim of the present invention is to provide a high-yield selective deposition of metallic compounds onto the front side of a substrate.

Another aim of the present invention is to provide further control of the anodic and cathodic half reaction of the electrochemical deposition techniques.

### SUMMARY OF THE INVENTION

The present invention relates to a bipolar "electroless" electrochemical process that solves the problems (low yield and self-limiting reactions) of existing electroless processes by galvanic displacement. It is different from the above "electrolytic" bipolar electrochemical processing as it does not need external feeder electrodes to separate the oxidation (anodic) and reduction (cathodic) half reactions.

Said bipolar electroless electrochemical processes according to the present invention refer to processes such as deposition, electro etching and surface modification reactions in general wherein galvanic displacement reactions (oxidation-reduction half reactions) are involved to achieve the desired electrochemical process.

In the following paragraphs reference is made to bipolar open-circuit deposition (Bi-OCD) but the invention is applicable to all bipolar open-circuit processes (Bi-OCP) in general, except the fact that the polarity of the used processes may change (e.g. anodic at the front side of the substrate for electro-etching or anodic at the back side of the substrate for deposition).

The present invention provides a method, referred to as photo Bi-OCD, for electroless deposition of metallic compounds onto the top surface of a semiconducting substrate comprising the following consecutive steps of:
- providing a semiconducting substrate having a first (e.g. front) side (surface) of said substrate and a second (e.g. back) side (surface) of said substrate preferably opposite to the firstside of said substrate thereby defining a thickness of semiconductor material,
- contacting the first side of the substrate with a first electrically conductive electrolyte comprising dissolved metal ions of the metallic compound,
- contacting the second side of the substrate with a second electrically conductive electrolyte,
- providing an electrical conductive path between the first and second electrolytes.

Said metallic compound comprises at least one metal or one metal alloy.

According to the invention, the metal compound can also comprise an alloy comprising more than one metal element.

Alloys can be classified by the number of their metal constituents. An alloy with two metal components is called a binary alloy; one with three metal components is a ternary alloy.

Two or more metal elements can be "co-deposited" in a method of the invention.

According to the invention, the term "co-deposition" means that two or more metal elements are deposited at a same time, from a same bath leading to an alloy.

Different aspects and types of "co-deposition" are known in state of the art and described e.g. by Brenner et al. in "Electrodeposition of Alloys", Academic Press, New York, 1963.

The alloy composition can be controlled by adjusting the bath composition (e.g. by changing the metal ion concentration), by adding complexing agents to bring the standard potentials closer together and/or using different deposition parameters (potential or current).

Preferably, said first side of the substrate is the processing front side, i.e. the side where the deposition occurs.

Said conductive electrolyte is a state of the art chemical solution comprising dissolved metal ions to produce an electrically conductive medium (Modern Electroplating (4th edition), M. Schlesinger and M. Paunovic (editors), Wiley, New York, 2000).

Preferably, said first and said second electrolytes are the same.

The present invention is based on the surprising observation that carrying out a method of the invention, comprising the differential illumination of the firstt side of said substrate versus the second side of said substrate, results in providing a driving force separating the cathodic and anodic partial reactions, starting a bipolar photo-electroless deposition and leading to high yield deposition of the metallic compound.

Said differential illumination is characterized by the fact that one side of the substrate (being the front side or the back side of the substrate) is more illuminated than the other side of the substrate (being the back side or the front side, respectively).

Preferably, the intensity of the illumination of the higher illuminated side of said substrate is at least 50% higher than the intensity of the illumination of the lower illuminated side of said substrate, more preferably the intensity of the illumination of the higher illuminated side of said substrate is 100% higher than the intensity of the illumination of the lower illuminated side of said substrate.

Preferably, a factor higher than 10⁴ and more preferably higher than 10⁵ between the intensity of illumination of the higher and lower illuminated sides is required.

Preferably, a differential illumination of the front side of the substrate versus the back side of the substrate is applied such that a driving force is created to separate the anodic (oxidation) and cathodic (reduction) partial reactions.

Preferably, the illuminance of said higher illuminated side of said substrate is higher than 10⁵ lux (lumen per square meter) and more preferably ranges between 10⁵ to 10⁹ lux.

Preferably, the illuminance of said lower illuminated side of said substrate is lower than 0.5 lux (lumen per square meter) and more preferably ranges between 10⁻⁵ to 0.1 lux.

Preferably, said illumination is carried out by natural, visible light up to UV light depending on the type of substrate, and his corresponding bandgap, used.

The wavelengths of said illumination preferably range between 100 nm and 700 nm, more preferably between 300 nm and 700 nm.

Said illumination can comprise a spectrum of wavelengths.

Monochromatic light can also be used in a method of the invention.

The oxidation-reduction half reactions are space separated on the front side of the substrate versus the back side of the substrate, such that the reduction half reaction or deposition occurs at the front side of the substrate and the oxidation half reaction occurs at the back side of the substrate.

The photo Bi-OCD process of the present invention can be used to deposit metallic nanoparticles onto a substrate. By choosing an appropriate pattern onto the substrate, said metallic nanoparticles can be selectively deposited onto the substrate. Said pattern can be a permanent pattern or a sacrificial pattern which can be removed in further processing steps.

The photo Bi-OCD process of the present invention can be used for the selective catalyst placement on semiconducting substrates to be used for growth and integration of nanowires (NW) or carbon nanotubes (CNT).

According to a preferred embodiment, the back side of said semiconducting substrate is more illuminated than its front side (the front side being at the same time possibly exposed to natural light of the ambient), in case said substrate is an n-type semiconducting substrate.

According to another preferred embodiment, the front side of said semiconduting substrate is more illuminated than its back side (the back side being at the same time possibly exposed to natural light of the ambient), in case said substrate is a p-type semiconducting substrate.

In case the substrate is a p-type semiconducting substrate, higher illumination is performed on the front side of the substrate to perform cathodic processing on the front side of the substrate (e.g. electrodeposition) and higher illumination is performed on the back side of the substrate to perform anodic processing on the front side of the substrate (e.g. electro etching).

In case the substrate is an n-type semiconducting substrate, the higher illumination is performed on the back side of the substrate to perform cathodic processing on the front side of the substrate (e.g. electrodeposition) and higher illumination is performed on the front side of the substrate to perform anodic processing on the front side of the substrate (e.g. electro etching).

As a preferred aspect, the present invention is related to a bipolar photo-electrochemical process for selective electroless processing such as the deposition of a metallic compound onto the top surface of a substrate, electro etching, electro polishing or substrate modification.

More preferably, according to the present invention, a selective photo Bi-OCD is performed where, prior to the steps of contacting the substrate to an electrically conductive electrolyte, a layer is provided defining a pattern on said substrate wherein e.g. openings (pores) are created to form said pattern.

Said pores or openings are not covered by the layer defining said pattern. As such, a direct contact between the metal deposited ions and the top surface of the substrate can occur.

Preferably said pattern is made of an insulating material to avoid electroless processing.

According to a preferred embodiment, the front side (top surface) of said substrate is at least partly covered with an insulating pattern whereby the deposition of the metallic compound takes place selectively into the openings not covered by said pattern.

Alternatively a metallic pattern can be first deposited onto the substrate such that the reduction half reaction or deposition occurs on the substrate inside the openings of the pattern and the oxidation half reaction occurs on the metal pattern itself (acting as anode) or vice versa.

Said metallic pattern can be a permanent or sacrificial pattern which can be removed or covered up in further processing.

According to another preferred embodiment, the top surface of the substrate is at least partly covered with a metal comprising pattern such that the deposition of the metallic compound takes place selectively onto the surface of the pattern in case the substrate is an n-type semiconducting substrate.

According to yet another preferred embodiment, the top surface of the substrate is at least partly covered with a metal comprising pattern such that the deposition of the metallic compound takes place selectively into the openings of the pattern in case the substrate is a p-type semiconducting substrate.

More preferably, in case said substrate is an n-type semiconducting substrate said substrate is selected from at least one of Si, Ge, GaAs doped with a group III element.

Preferably, said group III element is B, Al, Ga, In or Tl.

More preferably, in case said substrate is a p-type semiconducting substrate said substrate is selected from at least one of Si, Ge, GaAs doped with a group V element.

Preferably, said group V element is N, P, As, Sb or Bi.

Alternatively and also preferred, said substrate is a light sensitive metal oxide such as In₂O₃, TiO₂ or SnO₂.

In an alternative and also preferred embodiment a bipolar photo-electrochemical (photo Bi-OCD) process for selective electroless deposition is disclosed whereby the substrate is made of a semiconducting material (e.g. Si) and the pattern used to cover at least partly the front side of the substrate is made of a metallic compound. In this alternative and preferred embodiment, both oxidation and reduction (deposition) reactions take place at the front side of the substrate but separated by metal/semiconductor regions. Differential illumination is used to create a potential difference and the electrolyte solution makes contact with the front side of said substrate only (the back side of said substrate remains dry). For metal (alloy) deposition by the photo Bi-OCD process on the semiconductor substrate regions (i.e. semiconductor as cathode and metal as anode), the semiconductor substrate needs to be p-type and preferably the front side of the substrate is higher illuminated. For metal (alloy) deposition by the photo Bi-OCD process on the metallic regions (i.e. metal as cathode and semiconductor as anode), the front side of the substrate is higher illuminated and the substrate is an n-type semiconducting substrate. Further, the metallic regions are preferably inert to the dissolution (e.g. Ta, TaN, Ti, TiN, Pt).

In yet another alternative and also preferred embodiment a bipolar photo-electrochemical (photo Bi-OCD) process is disclosed whereby the semiconducting substrate is partly covered by metallic regions and the semiconducting regions are covered with an insulating pattern with openings exposing the semiconductor to the electrolyte. For a p-type semiconducting substrate, the exposed metallic regions will act as the anode and the exposed semiconductor as cathode upon illumination (preferably higher front illumination) leading to metal deposition by photo Bi-OCD on the semiconducting substrate. For an n-type semiconducting substrate, the exposed metallic regions will act as the cathode anode and the exposed semiconductor as anode upon illumination leading to electro-etching.

Examples of preferred semiconducting materials are group IV semiconductors, such as silicon (Si) and germanium (Ge), III-V semiconductors, such as GaAs, GaP, GaSb, InP, InSb, InAs and II-VI semiconductors such as ZnO, ZnS, CdS and CdSe. In case a semiconductor material (e.g. silicon) is used as substrate, said (silicon) substrate is preferably doped e.g. with group III elements (B, Al, Ga, In, Tl) causing the substrate (silicon) to function as an electron acceptor or in other words as a p-type substrate. Alternatively, the semiconductor material (e.g. silicon) is doped with group V elements (N, P, As, Sb, Bi) causing the substrate silicon to act as an electron donor or in other words as an n-type substrate. Therefore, a silicon substrate doped with boron creates a p-type semiconductor whereas one doped with phosphorus results in an n-type material. Another preferred example of a substrate is a GaAs consisting/containing material.

Alternatively light sensitive metal oxides can be used as substrate; preferred examples of these light sensitive metal oxides are In₂O₃, TiO₂ and SnO₂.

In case selective photo Bi-OCD is performed, a layer is deposited onto the front side of said substrate into which openings or pores are present and/or need to be created to form a pattern.

In a preferred embodiment said deposited layer is made of an insulating material or dielectric to avoid electrochemical deposition onto the surface of said layer.

Examples of said layer are oxides such as SiO₂ and alumina (aluminium oxide), nitrides such as Si₃N₅, carbides such as SiC, organic polymeric materials such as PMMA (polymethyl methacrylate) resists, low-k dielectric materials, zeolites such as silicates and porous oxides such as Anodized Alumina Oxide (AAO).

A SiO₂ layer can be deposited e.g. by Chemical Vapor Deposition (CVD) techniques.

In an alternative and also preferred embodiment said deposited layer is made of a metallic compound such as Ti, TiN, TaN, Ta, Al, Cr, Pb,... However in this alternative and preferred embodiment, both oxidation and deposition reactions may take place at the front side of the substrate but separated by metal/semiconductor.

Under illumination metal deposition (reduction) will occur in the semiconductor openings in case of a p-type semiconductor substrate and on the metal pattern in case of an n-type semiconducting substrate. The oxidation reaction will occur on the metallic pattern in case of a p-type substrate and in the semiconductor openings in case of an n-type semiconducting substrate.

In an alternative and also preferred embodiment, an insulating micro pattern may cover the macro patterned semiconductor and/or metallic regions. For example a rectangular area or box (e.g. 10 µm x 10 µm) of a p-type Si substrate is covered with a patterned SiO₂ with circular holes of 50 nm in diameter and a pitch of 100 nm exposing the p-site. This box is surrounded by a metal line (e.g. 500 nm wide TiN) on the Si substrate, forming a square around the Si/SiO₂ box.

Using said insulating pattern in the electroless photo Bi-OCD of the invention, the cathodic half reaction (reductive deposition) is confined to certain areas or holes i.e. limiting the place of deposition (referred to as "selective deposition") inside the holes of the pattern.

Preferably the openings (pores) in said deposited layer have a diameter of 1 nm up to several µm depending on the application. The openings are such that no insulating material is left at the bottom of the opening. The depth of the opening can range from 10 nm up to 500 nm depending on the application.

In case said deposited layer is made of a porous material such as zeolites or anodized alumina oxide (AAO), no patterning step is needed (but may be still used) to form pores (a pattern). The pores are instead formed by self-assembly.

Porous alumina (or AAO) can be formed on a substrate, such as silicon by iodization of an aluminum film deposited e.g. by means of Physical Vapor Deposition. This porous film can be from a few nanometers up to several microns thick.

Preferably, the front side of the substrate (comprising the pattern) is contacted to a first electrically conductive electrolyte comprising dissolved metal ions of the metallic compound to be deposited.

Preferably, the dissolved metal ions in the first electrically conductive electrolyte are capable of forming cathodic reactions on the front side of the substrate such that photo Bi-OCD of these metals onto the front side of the substrate is possible (inside openings in the dielectric or pores).

Preferred examples of these metal ions are Ni²⁺, Co²⁺, Cu²⁺, In³⁺, Au⁺, Au³⁺, Fe²⁺, Fe³⁺, Pt²⁺, Pd²⁺, Pb²⁺, Sb³⁺, Bi³⁺, Zn²⁺, Ga³⁺, Ge⁴⁺, Ru³⁺, Rh²⁺ and inorganic and organic complexes thereof, but the invention is not limited to these metals and can be applied to basically any material that can be electrodeposited, including alloys of these metals and in combination with W, Mo, V, Cr, Mn.

Preferred concentrations of the metals in the first electrically conductive electrolyte are in the range of 1mM up to 1M depending on the application.

Other ions added to the first electrically conductive electrolyte for complexation and improved conductivity are e.g. OH⁻, F⁻, Cl⁻, I⁻, Br⁻, NO₃⁻, SO₄²⁻, PO₄³⁻, S₂O₃²⁻, SO₃²⁻, sulfa mate-, flu borate-, borate-, cyanide-, fluoride- as anions and Na⁺, K⁺, Ca²⁺, Al³⁺, Mg²⁺, Li⁺, NH₄⁺, H⁺ as counter cations, with the total charge of anions and cations (including the metal ions) making a balance of zero.

Preferred concentrations of the salts in the first electrically conductive electrolyte are in the range of 1mM up to 6M depending on the application.

The electrolyte compositions are not limited to the above mentioned, and combinations are unlimited. For examples of recipes for typical plating electrolyte compositions is referred to literature.

The method of the present invention can also be extended to electrochemical processing in general such as electro etching or surface modification.

Preferably, the back side of the substrate is contacted to a second electrically conductive electrolyte. In this case, the substrate is separating the first and second electrolytes and we refer to "closed" photo Bi-OCD. Said separation can be made by mounting the substrate in-between two cells which have an opening sealed by the substrate (front side of said substrate seals the cell with electrolyte 1 and the back side of said substrate seals the cell with electrolyte 2). For fast loading and unloading of the substrate (wafer), a quick load/unload substrate (wafer) mount can be used which can contain one electrolyte and gets submerged in the second electrolyte or vice versa.

In case the substrate is a silicon containing substrate, said second electrically conductive electrolyte can contain HF or other fluoride containing compounds such as NH₄F, HBF₄ and combinations thereof (e.g. buffered HF) to avoid deposition of SiO₂ onto the back side of the substrate.

Preferred examples, but not limited to, of said second electrolyte are e.g. OH⁻, Cl⁻, NO³⁻, SO₄²⁻, PO₄³⁻, S₂O₃²⁻, SO₃²⁻, I⁻, I₃⁻, IO₃⁻, Br⁻, BrO₃⁻, sulfamate, fluoborate, borate, fluoride based solutions and mixtures thereof with counter cations of Na⁺, K⁺, Ca²⁺, Al³⁺, Li⁺, NH₄⁺, H⁺ (making the total ion balance = 0).

Preferred concentrations of the salts in the second electrolyte are in the range of 1mM up to 6M depending on the application.

Alternatively and also preferred, the substrate is fully immersed in said first electrically conductive electrolyte. In this case it is referred to as "open" photo Bi-OCD or open photo Bi-OCP and the anodic and cathodic reactions occur in the same electrolyte.

Alternatively and also preferred, only the front side of the substrate is immersed in said first electrically conductive electrolyte and the dry back side of the substrate is illuminated.

In case two electrolytes are needed, said first and second electrically conductive electrolytes are connected to each other by forming an electrical conductive path between the first and second electrolytes.

Said electrical conductive path can be created by means of a salt bridge or alternatively by means of external electrodes immersed in both electrolytes.

The closed photo Bi-OCD process starts as soon as the electrolytic contact is made between the two electrolytes.

In a preferred embodiment to perform selective photo Bi-OCD, light is used to create a potential difference between the front side of the substrate and the back side of the substrate and whereby the substrate is made of a semiconducting material (e.g. Si) and the pattern (if present) used to cover at least partly the front side of the substrate is made of an insulating material (to avoid deposition onto the pattern). In case an n-type semiconducting substrate is used, the back side of said substrate is more illuminated than the front side of said substrate. In case a p-type semiconducting substrate is used, the front side of said substrate is more illuminated than the back side of said substrate.

The above and other characteristics, features and advantages of the present invention will become apparent from the following detailed description, taken in conjunction with the accompanying drawings, which illustrate, by way of example, the principles of the invention. This description is given for the sake of example only, without limiting the scope of the invention. The reference figures quoted below refer to the attached drawings.

### DEFINITIONS

The term "electrochemical processes" as used in the present invention refer to both deposition processes and metal-removal processes (such as for example electro polishing, chemical etching and electro etching).

It is to be understood that in the present invention the terms "electrochemical processes" and "electrochemical processing" are equivalent.

The word "deposition" as used in the present invention means the act of depositing particles onto a surface of a substrate.

"Electrochemical processing" (ECP) and "electrochemical deposition" (ECD) as used in the present invention refer to an electrolytic process which requires an external voltage and current.

"Open-circuit processing" (OCP) and "open-circuit deposition" (OCD) as used in the present invention refer to electroless processing by galvanic displacement and electroless deposition by galvanic displacement respectively.

The respective bipolar processes as used in the present invention are bipolar electrochemical processing (Bi-ECP), bipolar electrochemical deposition (Bi-ECD), bipolar open-circuit processing (Bi-OCP) and bipolar open-circuit deposition (Bi-OCD).

The expression "electroless Bi-OCD" is a "photo Bi-OCD" process whereby light is used as a driving force to create the potential difference (i.e. photo voltage) between the front side of the substrate and the back side of the substrate.

It is to be understood that in the present invention the terms "electroless Bi-OCD", "photo Bi-OCD", "bipolar photo-OCD" and "photo-electroless Bi-OCD" are equivalent.

The term "selective deposition" onto a substrate as used in the present invention refers to the deposition of a compound on a predetermined specific area of a substrate and not on the whole substrate area.

It is to be understood that in the present invention the terms "electrochemical deposition" and "plating" are equivalent.

"Electroplating" as used in the present invention is the process of using electrical current to coat an electrically conductive object with a relatively thin layer of metal.

According to the invention, "electroless plating" means a non-galvanic type of plating method that involves several simultaneous reactions in an aqueous solution, which occur without the use of external electrical power.

The term "nanoparticle" as used in the present invention is a particle having a diameter which is preferably less than 100 nm.

The term "catalyst" as used in the present invention is a substance that accelerates the chemical reaction.

### BRIEF DESCRIPTION OF THE DRAWINGS

Exemplary embodiments are illustrated in referenced figures of the drawings. It is intended that the embodiments and figures disclosed herein are to be considered illustrative rather than restrictive.
Figure 1 (PRIOR ART) illustrates the metallic deposition in a pattern using unipolar OCD where both the front and back side of the substrate are exposed to light of the working environment.
Figure 2 illustrates the different processing steps according to the present invention to use bipolar photo-OCD to deposit a thick metallic layer on the top surface of an n-type substrate with more illumination on the back side of the substrate than on the front side of the substrate.
Figure 3 illustrates the different processing steps according to the present invention to use bipolar photo-OCD to deposit a thick metallic layer on the top surface of a p-type substrate with more illumination on the front side of the substrate than on the back side of the substrate.
Figure 4 illustrates the different processing steps according to the present invention to use bipolar photo-OCD to deposit a metallic compound into the inner pore openings of an insulating pattern situated on the top surface of an n-type substrate with more illumination on the back side of the substrate than on the front side of the substrate.
Figure 5 illustrates the different processing steps according to the present invention to use bipolar photo-OCD to deposit a metallic compound into the inner pore openings of a metallic pattern situated on the top surface of a p-type substrate with more illumination on the front side of the substrate than on the back side of the substrate.
Figure 6 illustrates the different processing steps according to the present invention to use bipolar photo-OCD to deposit a metallic compound onto the metallic pattern situated on the top surface of an n-type substrate with more illumination on the front side of the substrate than on the back side of the substrate.
Figure 7 illustrates the different processing steps according to the present invention to use bipolar photo-OCD to deposit a metallic compound into the inner pores of the insulating pattern situated on the top surface of a p-type substrate with more illumination on the front side of the substrate than on the back side of the substrate and wherein the top surface of the substrate further comprises a patterned metallic structure acting as anode.
Figure 8 illustrates a bipolar electrochemical set-up with two electrolyte baths using a salt bridge.
Figure 9 illustrates the band structure of the bipolar electrode. Figure 4A shows the electronic energy levels of a p-type substrate with higher illumination on the front side cathode of the substrate and Figure 4B shows the electronic energy levels of a bipolar n-type substrate with higher illumination on the back side anode of the substrate.
Figure 10 illustrates the selective photo-electroless Bi-OCD for gold (Au) deposition in patterned holes on SiO₂ in a dielectric layer on a p-type Si (100) substrate. The electrolyte used was 10mM Au(I) S₂O₃/SO₃ solution at room temperature and pH = 7.
Figure 11A illustrates (prior art) unipolar electroless electrochemical deposition compared to selective OCD (2-3 minutes OCD) as illustrated in Figure 11B of Au into the inner pores of the insulating pattern (150nm holes - pitch) on top surface of an n-type Si (100) substrate using a 10mM electrolyte solution (pH=7) .

### DETAILED DESCRIPTION OF ILLUSTRATIVE EMBODIMENTS

The present invention will be described with respect to particular embodiments and with reference to certain drawings but the invention is not limited thereto but only by the scope of the appended claims. The drawings described are only schematic and are non-limiting. In the drawings, the size of some of the elements may be exaggerated and not drawn to scale for illustrative purposes. The dimensions and the relative dimensions do not correspond to actual reductions to practice of the invention.

The invention will now be described by a detailed description of several embodiments of the invention. It is clear that other embodiments of the invention can be configured according to the knowledge of persons skilled in the art without departing from the true spirit or technical teaching of the invention, the invention being limited only by the terms of the appended claims.

In particular, the invention will be described with reference to the (selective) deposition of metallic compounds (e.g. nanoparticles for use a catalyst in nanowire or carbon nanotube growth), however, this is not intended to limit the invention, and is only one example of an application to perform the method of bipolar electrochemical processes according to the present invention.

It is appreciated to consider all electrochemical processes such as electro etching, electro polishing and surface modification as being part of the invention as well.

In the following detailed description reference is made to Bi-OCD but the invention is applicable to all Bi-OCP processes in general, except the fact that the polarity of the processes may change (e.g. anodic at the front side of the substrate for electro-etching).

The present invention discloses novel bipolar open-circuit processes (Bi-OCP) and bipolar open-circuit deposition (Bi-OCD) methods which makes use of light (illumination) to create a potential difference. Said novel bipolar processes are referred to as "photo Bi-OCP" and respectively "photo Bi-OCD".

A bipolar open-circuit deposition (Bi-OCD) process is disclosed for deposition of metallic compounds (pure metals or metal alloys) onto a substrate. By separating the oxidation-reduction half reactions a large and inexhaustible anode surface can be provided and the deposition process is free of surface oxide and not self-limiting leading to a high yield and unlimited thickness control.

The photo Bi-OCD process of the present invention can be used for the selective catalyst placement on semiconducting substrates to be used for growth and integration of nanowires (NW) or carbon nanotubes (CNT).

It is an advantage of the photo Bi-OCD process of the present invention to use Si based materials and process knowledge to realize the selective catalyst placement. The method can be easily processed and incorporated in current Si-based technology devices.

It is further an advantage of the photo Bi-OCD process of the present invention to avoid the need for a back contact (to be used as electrical terminal) onto the substrate. In many applications, direct contact to the substrate needs to be avoided to eliminate back side contamination. Using the method of the invention makes the use of (a) direct contact point(s) to the substrate needless and also other remedies such as implantation and/or metalization of the back side of the substrate are needless. Using the method of the invention makes it possible to use the electrolyte(s) as an electrical contact in which the substrate is acting as a bipolar electrode.

The present invention solves the problem of selective deposition of metallic compounds (pure metals or metal alloys) onto the front side of a substrate with high yield using a photo Bi-OCD process. The problem is solved first by covering the front side of the substrate with an insulating pattern such that the deposition of the metallic compound takes place selectively into the openings (pores) of said pattern and secondly by differential illumination of the front side of the substrate versus the back side of the substrate to provide a driving force to separate the cathodic and anodic partial reactions. More specifically, light is used to create a potential difference or photo voltage between the higher illuminated and lower illuminated areas. The photo Bi-OCD of the invention is further characterized as a bottom up electrochemical deposition process with high yield capable of filling very narrow pores (openings). Said openings can be in the nanometer range up to the micrometer range such that the method is suitable for use as catalyst placement for carbon nanotube (CNT) or nanowire (NW) growth as well as for through-hole plating processes where no physical contact can be made with the substrate.

The present invention further solves the problem of controlling the anodic and cathodic half reaction during electroless electrochemical processes such that the process becomes not self-limiting and a continuous process can be achieved with high yield. In case the electroless electrochemical process is a deposition (plating) process a continuous deposition of the compound of interest is achieved leading to thick deposits.

Thus, using the photo Bi-OCD of the invention makes it possible to deposit the metallic compound of interest inside the pattern with high yield, compared to a standard electroless electrochemical deposition (OCD) having poor control of the cathodic and anodic reactions and giving rise to low yield.

By using a preferred embodiment of the bipolar electroless approach of the present invention, the anodic and cathodic half reactions are separated using the back side of the substrate as a large inexhaustible anode surface.

The invention discloses further the use of more light or higher illumination of the back side (or alternatively of the front side) of the substrate to create a potential difference.

The invention is now described in more detail in different preferred embodiments or alternatives to perform the invention. Summarized a photo bipolar open-circuit process (photo Bi-OCP) is disclosed whereby a substrate having at least a front side of the substrate and a back side of the substrate is in contact with at least one electrolyte and the photo Bi-OCP process is performed onto the front side of the substrate using higher illumination of the back side (alternatively front side) of the substrate to achieve a potential difference.

In a preferred embodiment of the invention, a photo bipolar open-circuit deposition (photo Bi-OCD) *method for depositing a metallic layer* (pure metal or alloy of metals) onto a substrate is illustrated in Figure 2 for an n-type substrate and in Figure 3 for a p-type substrate. The method starts with the step of first providing a substrate **1.** Most preferred said substrate **1** is made of a p-type (or alternatively an n-type) semiconducting material and/or a light sensitive (metal) oxide and/or a semiconducting polymer.

Examples of preferred semiconducting materials are silicon (Si) and germanium (Ge). In case a semiconductor material (e.g. silicon) is used as substrate, said (silicon) substrate is preferably doped e.g. with group III elements (B, Al, Ga, In, Tl) causing the substrate (silicon) to function as an electron acceptor or in other words as a p-type substrate. Alternatively, the semiconductor material (e.g. silicon) is doped with group V elements (N, P, As, Sb, Bi) causing the substrate silicon to act as an electron donor or in other words as an n-type substrate. Therefore, a silicon substrate doped with boron creates a p-type semiconductor whereas one doped with phosphorus results in an n-type material. Another preferred example of a substrate is a GaAs consisting/containing material. Alternatively light sensitive metal oxides can be used as substrate, preferred examples of these light sensitive metal oxides are In₂O₃, TiO₂ and SnO₂.

In a next step, as illustrated in Figure 2B (and Figure 3B), the front side of the substrate is contacted to a first electrically conductive electrolyte comprising dissolved metal ions of the metallic compound to be deposited (indicated as solution 1).

Preferably, the dissolved metal ions (Mn⁺) in the first electrically conductive electrolyte are capable of forming cathodic reactions on the front side of the substrate such that photo Bi-OCP (deposition) of these metals onto the front side of the substrate is possible.

Preferred examples of these metals are Ni²⁺, Co²⁺, Cu²⁺, In³⁺, Au⁺, Fe²⁺, Fe³⁺, Pt²⁺, Pd²⁺,... but the invention is not limited to these metals and can be applied to basically anything that can be deposited.

Preferred concentrations of the metals in the first electrolyte are in the range of 1mM up to 1M depending on the application.

Preferred examples of said first electrolyte are e.g. Cl⁻, NO₃⁻, SO₄²⁻, PO₄³⁻, S₂O₃²⁻, SO₃²⁻, sulfamate, fluoborate, borate, cyanide, fluoride based solutions and mixtures thereof with counter cations of Na⁺, K⁺, Ca²⁺, Al³⁺, Li⁺, NH₄⁺, H⁺ (making the total ion balance = 0).

Preferred concentrations of the salts in the first electrolyte are in the range of 1mM up to 6M depending on the application.

Preferably, the back side of the substrate is contacted to a second electrically conductive electrolyte (indicated as solution 2). Said contact can be made by pressing the back side of the substrate to a porous path containing said second electrically conductive electrolyte or said contact can be clamped between two cells. In case the substrate is a silicon containing substrate, said second electrically conductive electrolyte can contain HF to avoid deposition of SiO₂ onto the back side of the substrate.

Preferred examples of said second electrolyte are e.g. Cl⁻, NO³⁻, SO₄²⁻, PO₄³⁻, S₂O₃²⁻, SO₃²⁻, sulfamate, fluoborate, borate, cyanide, fluoride based solutions and mixtures thereof with counter cations of Na⁺, K⁺, Ca²⁺, Al³⁺, Li⁺, NH₄⁺, H⁺ (making the total ion balance = 0).

Preferred concentrations of the salts in the second electrolyte are in the range of 1mM up to 6M depending on the application.

Said first and second electrolyte can be identical such that only one electrolytic bath is required and the substrate can be immersed in the bath.

In case two different (non-identical) electrolytes are needed, said first and second electrically conductive electrolytes are connected to each other by forming an electrical conductive path between the first and second electrolytes.

The electrical conductive path can be created by means of a salt bridge or alternatively by means of external electrodes immersed in both electrolytes.

Preferably, light **9** is used to achieve the potential difference needed to achieve photo Bi-OCD or in other words light is used as a driving force to create the potential difference between the front side of the substrate and the back side of the substrate. The light intensity of the incident light will determine the potential difference and the rate of reaction (more photo-electrons and photo holes available for reaction).

Natural, visible light up to UV light is used depending on the type of substrate, and his corresponding bandgap, used.

The wavelengths of said light range between 100 nm and 700 nm, preferably between 300 nm and 700 nm.

Said light can contain a spectrum of wavelengths.

Said light can be monochromatic light.

Examples of possible cathodic half reactions during the photo Bi-OCD process are:
**▪ Ni²⁺ +2e→Ni**
▪ **Co²⁺ +2e→Co**
▪ **Cu²⁺ +2e→Cu**
▪ **In³⁺ +3e→In**
▪ **Au⁺ +e→Au**

Examples of possible anodic half- reactions during photo Bi-OCD taking place at the back side of the substrate are:
▪ **Si + 4h⁺ + 2H₂0 → Sio₂⁻**
▪ **Si + 4h⁺ + 6F⁻ → SiF₆²⁻ (in the presence of HF)**

The above mentioned anodic and cathodic half reactions refer to displacement reactions with silicon (galvanic reaction) whereby silicon is oxidized and metal ions in solution are reduced and deposited onto the front side of the substrate. Said cathodic half reaction is highly selective for silicon surface.

The metal is first deposited as small metal nanoparticles **5** as illustrated in Figure 2C (or Figure 3C) and subsequently (longer OCD time) as a continuous metallic film **6** as illustrated in Figure 2D (or Figure 3D).

In a second preferred alternative of the first embodiment of the invention, a *method for selective depositing a metallic compound* (pure metal or alloy of metals) onto a substrate is disclosed and illustrated in Figure 4 for an n-type substrate. Said substrate is preferably selected from at least one of the preferred examples described above (according to the first preferred embodiment).

To achieve selective deposition of the metallic compound, the front side of the substrate **1** is partly covered with a pattern **3** to achieve selective electroless photo Bi-OCD.

Preferably said pattern is an insulating pattern such that no deposition of the metallic compound **5** results on the pattern **3** or in other words to avoid deposition onto the surface of said pattern **3.**

Said insulating pattern **3** can be created by first depositing a layer **2** onto the front side of the substrate **1** and subsequently (if needed) creating openings or pores **4** in said deposited layer to create a pattern. Preferably the openings (pores) **4** in said deposited layer have a diameter of 1 nm up to several µm depending on the application. The openings **4** are such that no insulating material is left at the bottom of the opening. The depth of the opening can range from 10 nm up to 500 nm depending on the application.

Preferably said deposited layer is made of an insulating material such as SiO₂ or organic polymeric materials.

A pattern (e.g. holes or pores but also lines or other shapes) can be created into said deposited layer by means of photolithographic patterning.

A SiO₂ layer can be deposited e.g. by Chemical Vapor Deposition techniques (CVD).

Alternatively and also preferred said deposited layer is made of a porous material such as zeolites or anodized alumina oxide (AAO) and no patterning step is needed to form pores (a pattern). The pores are instead formed by self-assembly.

Porous alumina (or AAO) can be formed on a substrate, such as silicon by anodization of an aluminum film deposited e.g. by means of Physical Vapor Deposition. This porous film can be from a few nanometers up to several microns thick.

After formation of the insulating pattern on the front side of the substrate differential illumination of the front side of the substrate versus the back side of the substrate is done to create a potential difference which separates the cathodic and anodic partial reactions.

In case the substrate is a p-type semiconducting substrate, the front side of the substrate is more illuminated **9** than the back side of the substrate and, in case the substrate is an n-type semiconducting substrate, the back side of the substrate is more illuminated **9** than the front side of the substrate. The metal is deposited into the pore openings as shown in Figure 4C.

The metal is first deposited as small metal nanoparticles **5** as illustrated in Figure 4C and if wanted the whole pattern (openings or holes) can be filled up with the metallic compound as illustrated in Figure 4D. The metal deposition continues with time until light is switched off.

Using the photo Bi-OCD of the invention makes it possible to deposit the metallic compound of interest inside the pattern with high yield, compared to standard electroless electrochemical plating having poor control of the cathodic and anodic reactions and giving rise to low yield as illustrated in Figure 1 and Figure 11A.

Figure 11A illustrates (prior art) unipolar electroless electrochemical deposition compared to selective OCD (2-3 minutes OCD) as illustrated in Figure 11B of Au into the inner pores of the insulating pattern (150 nm holes - pitch) on top surface of an n-type Si (100) substrate using a 10mM electrolyte solution (pH=7). It is noticed from these 2 figures that the yield of the selective OCD (illustrated in Figure 11B) compared to the yield of the prior art unipolar electroless electrochemical deposition (Figure 11A) is at least doubled.

Full illumination is needed to achieve good uniformity of deposition.

In a third and also preferred alternative of the above described embodiments as shown in Figure 5 and Figure 6 said deposited layer to create a pattern on the front side of the substrate is made of a metallic compound. Said substrate is preferably selected from at least one of the preferred examples described above (according to the first preferred embodiment). However in this alternative and preferred embodiment, both oxidation and deposition reactions take place at the front side of the substrate but separated by metal/semiconductor regions having deposition on the metallic regions or alternatively onto the metallic pattern (using the metallic pattern as anode).

Using said metallic pattern onto a p-type substrate in the photo Bi-OCD of the invention, the *anodic half reaction* can be confined onto the metallic pattern i.e. limiting the place of deposition (referred to as "selective deposition") inside the holes **33** of the metallic pattern **32** as shown in Figure 6. The metallic pattern **32** is then acting as anode instead of the back side of the substrate **1** such that only the front side of the (p-type) substrate **1** needs to be in contact with the electrolyte (only one electrolyte is required) and deposition is taking place inside **32** the pattern onto the front side of the p-type substrate **1.**

Alternatively, in case of an n-type substrate, *the cathodic half reaction* is confined to selectively onto the metallic pattern **32** limiting the place of deposition (referred to as "selective deposition") onto the metallic pattern **32** as shown in Figure 5. The openings (holes) **33** in between the metallic pattern are then acting as anode instead of the back side of the substrate **1** such that only the front side of the substrate **1** needs to be in contact with the electrolyte (only one electrolyte is required) and deposition of the metallic compound **35** is taking place onto the metallic pattern **32** onto the front side of the substrate and the openings **34** are acting as anode.

After covering the front side of the substrate with a metallic pattern such that the deposition of the metallic compound takes place selectively into the openings (pores) of said pattern or onto the pattern, higher illumination **9** of the front side of the substrate is performed to provide a driving force to separate the cathodic and anodic partial reactions. More specifically light is used to create a potential difference.

In case a p-type semiconducting substrate is used, the front side of said substrate is more illuminated **9** than the back side of the substrate and the deposition is taking place inside the metallic pattern onto the front side of the p-type substrate as shown in Figure 6. In case an n-type semiconducting substrate is used, the front side of said substrate is more illuminated **9** than the back side of the substrate and deposition of the metallic compound **35** is taking place onto the metallic pattern as shown in figure 5.

In a fourth and also preferred alternative of the above described embodiments and as shown in Figure 7 *an extra structure* is deposited onto the front side of the substrate, said extra structure is then acting as an anode and both oxidation and deposition reactions take place at the front side of the substrate such that only the front side of the substrate is in contact with the electrolytic solution.

In Figure 7 an extra metal comprising structure **40** (e.g. comprising Ti (TiN), Ta (TaN), W, ...) is present on the front side of the substrate **1.** Said substrate **1** is selected from a p-type semiconducting material as described in the first preferred embodiment. Said extra metal comprising structure **40** is then acting as an anode and both oxidation and deposition reactions take place at the front side of the substrate such that only the front side of the substrate is in contact with the electrolytic solution.

To realize a selective deposition onto the substrate **1** of the metallic compound, the front side of the substrate **1** is partly covered with an insulating pattern **32** to achieve a selective photo Bi-OCD process. Said pattern is an insulating pattern **32** as described in the second preferred embodiment above such that no deposition of the metallic compound **35** is achieved on the pattern **32** or in other words to avoid deposition onto the surface of said pattern **32.**

Most preferred, higher illumination **9** on the front side of the substrate is performed to provide a driving force to separate the cathodic and anodic partial reactions.

Alternatively, higher illumination **9** on the back side of the substrate is performed to separate the cathodic and anodic partial reactions.

The illuminance of the higher illuminated side of the substrate is higher than 10⁵ lux (lumen per square meter) and preferably ranges between 10⁵ to 10⁹ lux.

The illuminance of the lower illuminated side of the substrate is lower than 0.5 lux (lumen per square meter) and preferably ranges between 10⁻⁵ to 0.1 lux.

More specifically light is used to create a potential difference.

### EXAMPLES

### Example 1: selective photo-electroless Bi-ECP of gold in patterned silicon via holes.

Figure 7 illustrates the selective photo-electroless Bi-ECP for gold deposition in patterned silicon via holes. Gold (Au) was deposited on SiO₂ in patterned contact holes on a p-type Si (100) substrate. The electrolyte used was 10mM Au(I) S₂O₃/SO₃ solution at room temperature (e.g. T=21°C) and pH = 7.

## Claims

1. A method, referred to as photo Bi-OCD, for electroless deposition of a metallic compound onto the top surface of a semiconducting substrate comprising the following consecutive steps of:
- providing a semiconducting substrate (1) having a first side (100) of said substrate and a second side (110) of said substrate preferably opposite to the first side of said substrate thereby defining a thickness of semiconductor material,
- contacting the first side of the substrate with a first (10) electrically conductive electrolyte comprising dissolved metal ions of the metallic compound,
- contacting the second side of the substrate with a second (11) electrically conductive electrolyte,
- providing an electrical conductive path between said first (10) and second (11) electrolytes,
**characterized in that**:
- the firstt side of said substrate versus the second side of said substrate is differential illuminated for creating a potential difference between said first and said second side of said substrate.

2. The method according to claim 1, wherein for an n-type semiconducting substrate the back side (14) of said substrate is more illuminated than the front side of said substrate.

3. The method according to claim 1, wherein for a p-type semiconducting substrate the front side (15) of said substrate is more illuminated than the back side of said substrate.

4. The method according to any one of the preceding claims, wherein the intensity of the illumination of the higher illuminated side of said substrate is at least 50% higher than the intensity of the illumination of the lower illuminated side of said substrate, more preferably the intensity of the illumination of the higher illuminated side of said substrate is 100% higher than the intensity of the illumination of the lower illuminated side of said substrate.

5. The method according to any one of the preceding claims, to perform a selective photo Bi-OCD whereby the method further comprises, prior to the steps of contacting the substrate to an electrically conductive electrolyte, the step of providing on said substrate (1) a layer (2) into which openings are created to form a pattern (3).

6. The method according to any one of the preceding claims, whereby said photo Bi-OCD is a selective photo Bi-OCD whereby the first side of the substrate (1) is at least partly covered with an insulating pattern (3) such that the deposition of the metallic compound takes place selectively into the openings of the pattern (3).

7. The method according to claim 6, whereby said insulating pattern is made of a material comprising oxides such as alumina, organic polymeric materials, low-k dielectric materials, zeolites and porous oxides (AAO).

8. The method according to claim 6 or 7, whereby said photo Bi-OCD is a selective photo Bi-OCD whereby the first side surface of the substrate (1) is at least partly covered with a metal comprising pattern (32) such that the deposition of the metallic compound takes place:
- selectively onto the surface of the pattern (32) in case the substrate is an n-type semiconducting substrate
- selectively into the openings of the pattern in case the substrate is a p-type semiconducting substrate.

9. The method of claim 8, whereby said metal comprising pattern is selected from metals such as TiN, TaN, or w.

10. The method according to any one of the preceding claims, whereby said substrate is an n-type semiconducting substrate selected from at least one of Si, Ge, GaAs doped with a group III element such as B, Al, Ga, In, or Tl.

11. The method according to any one of the preceding claims, whereby said substrate is a p-type semiconducting substrate selected from at least one of Si, Ge, GaAs doped with a group V element such as N, P, As, Sb, or Bi.

12. The method according to any one of the preceding claims, whereby said substrate is a light sensitive metal oxide such as In₂O₃, TiO₂, or SnO₂.

13. The method according to any one of the preceding claims, whereby said first electrically conductive electrolyte (10) comprises dissolved metal ions such as Ni²⁺, Co²⁺, Cu²⁺, In³⁺, Au⁺, Au³+, Fe²⁺, Fe³⁺, Pt²⁺, Pd²⁺, Pb²⁺, Sb³⁺, Bi³⁺, Zn²⁺, Ga³⁺, Ge⁴⁺, Ru³⁺, Rh²⁺, inorganic and organic complexes thereof, alloys of these metals and in combination with W, Mo, V, Cr or Mn.

14. The method of claim 13, whereby the concentrations of said metal ions in said first electrically conductive electrolyte (10) are in the range of 1mM up to 1M.

15. The method according to any one of the preceding claims, whereby said second electrically conductive electrolyte (11) comprises anions of the group of OH⁻, Cl⁻, NO³⁻, SO₄²⁻, PO₄³⁻ , S₂O₃²⁻, SO₃²⁻, I⁻, I₃⁻, IO₃⁻, Br⁻, BrO₃⁻, sulfamate, fluoborate, borate, fluoride based solutions and mixtures thereof with counter cations of Na⁺, K⁺, Ca²⁺, Al³⁺, Li⁺, NH₄⁺, H⁺.

16. The method according to claim 15, whereby the concentrations of the anionsin said second electrically conductive electrolyte (11) are in the range of 1mM up to 6M.

17. The method according to any one of the preceding claims,whereby said electrical conductive path between the first and second conductive electrolytes is performed using a salt bridge.

18. The methods according to any one of the preceding claims 5 to 17, whereby the first side of the substrate is more illuminated than the second side of the substrate and the first side of the substrate (1) further comprises an extra metallic comprising structure (940) to act as anode in the photo Bi-OCD such that only the first side of the substrate (1) is contacted to said first (10) electrically conductive electrolyte comprising dissolved metal ions of the metallic compound (keeping the back side of the substrate dry) and such that the deposition of the metallic compound takes place selectively into the openings of the insulating pattern (32).

19. The method of claim 18, whereby the substrate is a p-type semiconducting substrate.

20. Use of the method according to any one of the preceding claims 1 to 19 for a selective deposition of metallic nanoparticles used as catalyst for growth of semiconductor nanowires (NW) or carbon nanotubes (CNT).

## Patentansprüche

1. Verfahren, das als Photo-Bi-OCD bezeichnet wird, zum stromlosen Abscheiden einer metallischen Verbindung auf die obere Oberfläche eines Halbleitersubstrats, das die nachstehenden aufeinanderfolgenden Schritte umfasst:
- Bereitstellen eines Halbleitersubstrats (1) mit einer ersten Seite (100) des Substrats und einer zweiten Seite (110) des Substrats, die der ersten Seite des Substrats vorzugsweise gegenüberliegt, wodurch eine Dicke eines Halbleitermaterials definiert wird,
- Inkontaktbringen der ersten Seite des Substrats mit einem ersten (10) elektrisch leitenden Elektrolyten, umfassend aufgelöste Metallionen der metallischen Verbindung,
- Inkontaktbringen der zweiten Seite des Substrats mit einem zweiten (11) elektrisch leitenden Elektrolyten,
- Bereitstellen eines elektrisch leitenden Wegs zwischen dem ersten (10) und dem zweiten (11) Elektrolyten,
**dadurch gekennzeichnet, dass**:
- die erste Seite des Substrats im Vergleich zur zweiten Seite des Substrats unterschiedlich beleuchtet wird, um einen potenziellen Unterschied zwischen der ersten und der zweiten Seite des Substrats zu bilden.

2. Verfahren nach Anspruch 1, wobei die Rückseite (14) des Substrats für ein n-Typ-Halbleitermaterial stärker als die Vorderseite des Substrats beleuchtet wird.

3. Verfahren nach Anspruch 1, wobei die Vorderseite (15) des Substrats für ein p-Typ-Halbleitermaterial stärker als die Rückseite des Substrats beleuchtet wird.

4. Verfahren nach einem der vorstehenden Ansprüche, wobei die Intensität der Beleuchtung der stärker beleuchteten Seite des Substrats zumindest um 50 % höher als die Intensität der Beleuchtung der schwächer beleuchteten Seite des Substrats ist, mehr bevorzugt die Intensität der Beleuchtung der stärker beleuchteten Seite des Substrats 100 % höher als die Intensität der Beleuchtung der schwächer beleuchteten Seite des Substrats ist.

5. Verfahren nach einem der vorstehenden Ansprüche, um eine selektive Photo-Bi-OCD durchzuführen, wobei das Verfahren ferner vor den Schritten des Inkontaktbringens des Substrats mit einem elektrisch leitenden Elektrolyten den Schritt des Bereitstellens einer Schicht (2) auf dem Substrat (1) umfasst, in der Öffnungen gebildet werden, um ein Muster (3) zu bilden.

6. Verfahren nach einem der vorstehenden Ansprüche, wobei die Photo-Bi-OCD eine selektive Photo-Bi-OCD ist, wobei die erste Seite des Substrats (1) zumindest teilweise mit einem Isoliermuster (3) bedeckt ist, so dass das Abscheiden der metallischen Verbindung selektiv in die Öffnungen des Musters (3) erfolgt.

7. Verfahren nach Anspruch 6, wobei das Isoliermuster aus einem Material hergestellt ist, das Oxide wie z. B. Aluminiumoxid, organische polymere Materialien, Low-k dielektrische Materialien, Zeolithen und poröse Oxide (AAO) umfasst.

8. Verfahren nach Anspruch 6 oder 7, wobei die Photo-Bi-OCD eine selektive Photo-Bi-OCD ist, wobei die erste Seitenfläche des Substrats (1) zumindest teilweise mit einem metallumfassenden Muster (32) bedeckt ist, so dass das Abscheiden der metallischen Verbindung erfolgt:
- selektiv auf die Oberfläche des Musters (32), wenn das Substrat ein n-Typ-Halbleitersubstrat ist,
- selektiv in die Öffnungen des Musters, wenn das Substrat ein p-Typ-Halbleitersubstrat ist.

9. Verfahren nach Anspruch 8, wobei das metallumfassende Muster aus Metallen wie z. B. TiN, TaN, oder W ausgewählt ist.

10. Verfahren nach einem der vorstehenden Ansprüche, wobei das Substrat ein n-Typ-Halbleitersubstrat ist, das aus zumindest einem von Si, Ge, GaAs, dotiert mit einem Gruppe-III-Element wie z. B. B, Al, Ga, In, oder Tl ausgewählt ist.

11. Verfahren nach einem der vorstehenden Ansprüche, wobei das Substrat ein p-Typ-Halbleitersubstrat ist, das aus zumindest einem von Si, Ge, GaAs, dotiert mit einem Gruppe-V-Element wie z. B. N, P, As, Sb, oder Bi ausgewählt ist.

12. Verfahren nach einem der vorstehenden Ansprüche, wobei das Substrat ein lichtempfindliches Metalloxid wie z. B. In₂O₃, TiO₂, oder SnO₂ ist.

13. Verfahren nach einem der vorstehenden Ansprüche, wobei der erste elektrisch leitende Elektrolyt (10) aufgelöste Metallionen wie z. B. Ni²⁺, Co²⁺, Cu²⁺, In³⁺, Au⁺, Au³⁺, Fe²⁺, Fe³⁺, Pt²⁺, Pd²⁺, Pb²⁺, Sb³⁺, Bi³⁺, Zn²⁺, Ga³⁺, Ge⁴⁺, Ru³⁺, Rh²⁺, anorganische und organische Komplexe davon, Legierungen dieser Metalle und in Kombination mit W, Mo, V, Cr oder Mn umfasst.

14. Verfahren nach Anspruch 13, wobei die Konzentrationen der Metallionen im ersten elektrisch leitenden Elektrolyten (10) im Bereich von 1 mM bis 1 M liegen.

15. Verfahren nach einem der vorstehenden Ansprüche, wobei der zweite elektrisch leitende Elektrolyt (11) Anionen der Gruppe von OH⁻, Cl⁻, NO³⁻, SO₄²⁻, PO₄³⁻, S₂O₃²⁻, SO₃²⁻, I⁻, I₃⁻, IO₃⁻, Br⁻, BrO₃⁻, Sulfamat, Fluoborat, Borat, fluoridbasierten Lösungen und Mischungen davon mit Gegenionen von Na⁺, K⁺, Ca²⁺, Al³⁺, Li⁺, NH₄⁺, H⁺ umfasst.

16. Verfahren nach Anspruch 15, wobei die Konzentrationen der Anionen im zweiten elektrisch leitenden Elektrolyten (11) im Bereich von 1 mM bis 6 M liegen.

17. Verfahren nach einem der vorstehenden Ansprüche, wobei der elektrisch leitende Weg zwischen dem ersten und dem zweiten leitenden Elektrolyten unter Verwendung einer Salzbrücke durchgeführt wird.

18. Verfahren nach einem der vorstehenden Ansprüche 5 bis 17, wobei die erste Seite des Substrats stärker als die zweite Seite des Substrats beleuchtet wird und die erste Seite des Substrats (1) ferner eine zusätzliche metallumfassende Struktur (940) umfasst, die bei der Photo-Bi-OCD als Anode agiert, so dass nur die erste Seite des Substrats (1) mit dem ersten (10) elektrisch leitenden Elektrolyten in Kontakt gebracht wird, der aufgelöste Metallionen der metallischen Verbindung umfasst (wobei die Rückseite des Substrats trocken gehalten wird) und so dass das Abscheiden der metallischen Verbindung selektiv in die Öffnungen des Isoliermusters (32) erfolgt.

19. Verfahren nach Anspruch 18, wobei das Substrat ein p-Typ-Halbleitersubstrat ist.

20. Verwendung des Verfahren nach einem der vorstehenden Ansprüche 1 bis 19 zum selektiven Abscheiden von metallischen Nanopartikeln, die als Katalysator zum Züchten von Halbleiternanodrähten (NW) oder Kohlenstoffnanoröhrchen (CNT) verwendet werden.

## Revendications

1. Procédé, appelé Bi-OCD photo, de dépôt autocatalytique d'un composé métallique sur la surface supérieure d'un substrat semi-conducteur comprenant les étapes consécutives suivantes :
- la fourniture d'un substrat semi-conducteur (1) ayant un premier côté (100) dudit substrat et un second côté (110) dudit substrat de préférence opposé au premier côté dudit substrat, définissant ainsi une épaisseur de matériau semi-conducteur,
- la mise en contact du premier côté du substrat avec un premier (10) électrolyte électroconducteur comprenant des ions métalliques dissous du composé métallique,
- la mise en contact du second côté du substrat avec un second (11) électrolyte électroconducteur,
- la fourniture d'un trajet électroconducteur entre lesdits premier (10) et second (11) électrolytes,
**caractérisé en ce que**
- le premier côté dudit substrat reçoit un éclairage différentiel par rapport au second côté dudit substrat pour créer une différence de potentiel entre ledit premier et ledit second côté dudit substrat.

2. Procédé selon la revendication 1, dans lequel pour un substrat semi-conducteur de type n, le côté arrière (14) dudit substrat est plus éclairé que le côté avant dudit substrat.

3. Procédé selon la revendication 1, dans lequel pour un substrat semi-conducteur de type p, le côté avant (15) dudit substrat est plus éclairé que le côté arrière dudit substrat.

4. Procédé selon l'une quelconque des revendications précédentes, dans lequel l'intensité de l'éclairage du côté plus éclairé dudit substrat est au moins 50 % plus élevée que l'intensité d'éclairage du côté moins éclairé dudit substrat, plus préférablement l'intensité de l'éclairage du côté plus éclairé dudit substrat est 100 % plus élevée que l'intensité de l'éclairage du côté moins éclairé dudit substrat.

5. Procédé selon l'une quelconque des revendications précédentes, destiné à effectuer un Bi-OCD photo sélectif, le procédé comprenant en outre, en plus des étapes de mise en contact du substrat avec un électrolyte électroconducteur, l'étape consistant à prévoir sur ledit substrat (1) une couche (2) dans laquelle des ouvertures sont créées pour former un motif (3).

6. Procédé selon l'une quelconque des revendications précédentes, dans lequel ledit Bi-OCD photo est un Bi-OCD photo sélectif, dans lequel le premier côté du substrat (1) est au moins partiellement couvert d'un motif isolant (3) de telle sorte que le dépôt du composé métallique a lieu sélectivement dans les ouvertures du motif (3).

7. Procédé selon la revendication 6, dans lequel ledit motif isolant est constitué d'un matériau comprenant des oxydes tels que de l'alumine, des matériaux polymères organiques, des matériaux diélectriques à faible k, des zéolites et des oxydes poreux (AAO).

8. Procédé selon la revendication 6 ou 7, dans lequel ledit Bi-OCD photo est un Bi-OCD photo sélectif, dans lequel la première surface latérale du substrat (1) est au moins partiellement couverte d'un métal comprenant un motif (32) de telle sorte que le dépôt du composé métallique a lieu :
- sélectivement sur la surface du motif (32) lorsque le substrat est un substrat semi-conducteur de type n
- sélectivement dans les ouvertures du motif lorsque le substrat est un substrat semi-conducteur de type p.

9. Procédé selon la revendication 8, dans lequel ledit métal comprenant le motif est choisi parmi des métaux tels que TiN, TaN ou W.

10. Procédé selon l'une quelconque des revendications précédentes, dans lequel ledit substrat est un substrat semi-conducteur de type n choisi parmi au moins un de Si, Ge, GaAs dopé avec un élément de groupe III tel que B, Al, Ga, In ou Tl.

11. Procédé selon l'une quelconque des revendications précédentes, dans lequel ledit substrat est un substrat semi-conducteur de type p choisi parmi au moins un de Si, Ge, GaAs dopé avec un élément de groupe V tel que N, P, As, Sb ou Bi.

12. Procédé selon l'une quelconque des revendications précédentes, dans lequel ledit substrat est un oxyde métallique sensible à la lumière tel que In₂O₃, TiO₂ ou SnO₂.

13. Procédé selon l'une quelconque des revendications précédentes, dans lequel ledit premier électrolyte électroconducteur (10) comprend des ions métalliques dissous tels que Ni²⁺, Co²⁺, Cu²⁺, In³⁺, Au⁺, Au³⁺, Fe²⁺, Fe³⁺, Pt²⁺, Pd²⁺, Pb²⁺, Sb³⁺, Bi³⁺, Zn²⁺, Ga³⁺, Ge⁴⁺, Ru³⁺, Rh²⁺, des complexes inorganiques et organiques de ceux-ci, des alliages de ces métaux et en combinaison avec W, Mo, V, Cr ou Mn.

14. Procédé selon la revendication 13, dans lequel les concentrations desdits ions métalliques dans ledit premier électrolyte électroconducteur (10) sont dans la plage de 1 mM jusqu'à 1 M.

15. Procédé selon l'une quelconque des revendications précédentes, dans lequel ledit second électrolyte électroconducteur (11) comprend des anions du groupe OH⁻, Cl⁻, NO³⁻, SO₄²⁻, PO₄³⁻, S₂O₃²⁻, SO₃²⁻, I⁻, I₃⁻, IO₃⁻, Br⁻, BrO₃⁻, des solutions à base de sulfamate, fluoborate, borate, fluorure et leurs mélanges avec des contre-cations de Na⁺, K⁺, Ca²⁺, Al³⁺, Li⁺, NH₄⁺, H⁺.

16. Procédé selon la revendication 15, dans lequel les concentrations des anions dans ledit second électrolyte électroconducteur (11) sont dans la plage de 1 mM à 6 M.

17. Procédé selon l'une quelconque des revendications précédentes, dans lequel ledit trajet électroconducteur entre les premier et second électrolytes conducteurs est réalisé au moyen d'un pont de sel.

18. Procédés selon l'une quelconque des revendications 5 à 17 précédentes, dans lesquels le premier côté du substrat est plus éclairé que le second côté du substrat et le premier côté du substrat (1) comprend en outre une structure métallique supplémentaire (940) destinée à servir d'anode dans le Bi-OCD photo de telle sorte que seul le premier côté du substrat (1) est en contact avec ledit premier (10) électrolyte électroconducteur comprenant les ions métalliques dissous du composé métallique (laissant le côté arrière du substrat sec) et de telle sorte que le dépôt du composé métallique a lieu sélectivement dans les ouvertures du motif isolant (32).

19. Procédé selon la revendication 18, dans lequel le substrat est un substrat semi-conducteur de type p.

20. Utilisation du procédé selon l'une quelconque des revendications 1 à 19 précédentes pour un dépôt sélectif de nanoparticules métalliques utilisées comme catalyseur pour la croissance de nanofils semi-conducteurs (NW) ou de nanotubes de carbone (CNT).
